

## 1

3,075,899

### BATHS FOR THE PRODUCTION OF METAL ELECTROPLATES

Wennemar Strauss and Wolf-Dieter Willmund, Dusseldorf-Holthausen, Germany, assignors to Dehydag, Deutsche Hydrierwerke G.m.b.H., Dusseldorf, Germany, a corporation of Germany

No Drawing. Filed Apr. 20, 1959, Ser. No. 807,290  
Claims priority, application Germany Apr. 26, 1958  
12 Claims. (Cl. 204—52)

This invention relates to a method and bath for obtaining bright metal electrodeposits. It more particularly relates to the use of sulfonic acid derivatives of thioamides or isothioamides for obtaining bright metal electrodeposits.

From German Patent No. 837,029, it is known that acid copper baths can be improved by the addition of thioacetamide as a brightening agent. It was found, however, that the brightening effect achieved thereby is only moderate. The subsequent polishing of the electroplated objects requires a separate step and it is connected with a considerable abrasion of the previous applied copper deposits.

It is an object of this invention to provide a method and bath for obtaining bright metal electrodeposits which require no mechanical polishing.

Another object of this invention is to provide electroplating bath brightener compounds which have high stability and long life.

It is a further object to provide a method for producing electroplating brightener compounds.

These and other objects of our invention will become apparent as the description thereof proceeds.

We have now found that the brightening effect on electrodeposited metal, and particularly copper plates, can be substantially improved, whereby a subsequent polishing step becomes, as a rule, completely superfluous, by adding to the acid electroplating bath acyclic or cyclic thioamides or isothioamides, which contain a sulfonic acid group which is attached to the nitrogen atoms of the thioamide or isothioamide through a hydrocarbon radical. These compounds are sufficiently soluble in the electroplating baths, very stable and are only very slowly consumed in these baths.

The compounds used as brightening agents in accordance with the invention have the general structural formulas



and



wherein R, R' and R'', represent hydrocarbon radicals, and R and/or R' may also be hydrogen atoms. R and R' may further form a polymethylene chain, so that the thioamide group is a member of a heterocyclic ring. The hydrocarbon radicals are R' and R'', may carry

## 2

substituents such as halogen, cyano, thiocyanato and/or hydroxyl groups, or they may also be interrupted by heteroatoms or heteroatom groups, and they may particularly contain additional thioamide and isothioamide groups. Brightening agents of this type are, for example, the water soluble salts of the following compounds:

- Thioacetamide-N-(methane-sulfonic acid),
- Thioformamide-N-(propane- $\omega$ -sulfonic acid),
- Thioacetamide-N-(propane- $\omega$ -sulfonic acid),
- Thiopropionamide-N-(propane- $\omega$ -sulfonic acid),
- Thiobutyramide-N-(propane- $\omega$ -sulfonic acid),
- Thioformamide-N-(butane- $\omega$ -sulfonic acid),
- Thiobutyramide-N-(butane- $\omega$ -sulfonic acid),
- Thioacetamide-N-(isohexane- $\omega$ -sulfonic acid),
- Thioacetamide-N-(toluole-2-sulfonic acid),
- Thiopropionamide-N-(naphthalene-8-sulfonic acid),
- Thioacetamide-N-ethyl-N-(propane- $\omega$ -sulfonic acid),
- Thiopropionamide-N-propyl-N-(propane- $\omega$ -sulfonic acid),
- Thioacetamide-N-butyl-N-(propane- $\omega$ -sulfonic acid),
- Thioacetamide-N-phenyl-N-(propane- $\omega$ -sulfonic acid),
- Thioacetamide-N-benzyl-N-(propane- $\omega$ -sulfonic acid),
- Thioacetamide-N-cyclohexyl-N-(propane- $\omega$ -sulfonic acid),
- Thiobenzamide-N-(propane- $\omega$ -sulfonic acid),
- 2-hydroxy-thiobenzamide-N-(propane- $\omega$ -sulfonic acid),
- Thionaphthamide-N-(propane- $\omega$ -sulfonic acid),
- Thioacetamide-N-( $\beta$ -hydroxyethyl)-N-(propane- $\omega$ -sulfonic acid),
- Thioacetamide-N-(2-hydroxypropane- $\omega$ -sulfonic acid),
- Thioacetamide-N-(2-chloropropane- $\omega$ -sulfonic acid),
- Ethylene-1,2-bis-[thioacetamide-N,N'-bis-(propane- $\omega$ -sulfonic acid)-N,N'],
- Ethylene-1,2-bis-[thioacetamide-N,N'-bis-(butane- $\omega$ -sulfonic acid)-N,N'],
- Butyrothiolactam-N-(propane- $\omega$ -sulfonic acid),
- Valerothiolactam-N-(propane- $\omega$ -sulfonic acid),
- Caprothiolactam-N-(propane- $\omega$ -sulfonic acid),
- Caprothiolactam-N-(butane- $\omega$ -sulfonic acid),
- N-(propane- $\omega$ -sulfonic acid)-thioacetimino-S-ethylester,
- N-(butane- $\omega$ -sulfonic acid)-thiobenzimino-S-n-butylester,
- Thiopicolinic acid - N - methyl - N - (propane -  $\omega$  - sulfonic acid)-amide-N'-(propane- $\omega$ -sulfonic acid)butane,
- Thiopicolinic acid-N-phenyl-N-(propane- $\omega$ -sulfonic acid)-amide-N'-(propane- $\omega$ -sulfonic acid)butane,

The production of these compounds takes place, for example by reaction of the thioamides or isothioamide-S-esters with organic amino sulfonic acids or their salts. The isothioamide-S-esters may also be reacted with haloalkanesulfonic acids or sultones. Suitable sulfonic acids are primarily those of the aliphatic or aromatic series which react with the thioamides or isothioamides in aqueous or non-aqueous, for example in alcoholic solution or suspension. The reaction with the sultones may also take place in the molten state. The reactions proceed readily and smoothly and as a rule produce high yields, so that the end product may be used as such, possibly after neutralization, and advantageously in the form of corresponding aqueous solutions.

In order to broaden the effective range of the working temperature in acid baths, thioamides or isothioamides which generally contain no sulfonic acid groups may be simultaneously used. In this manner the working temperature may be increased up to 55° C. and

higher without unfavorably influencing the brightness and ductility of the electrodeposits. In addition, other known brightening agents may also be added to these electroplating baths.

In some cases it is recommended to use simultaneously wetting agents and ductility improving agents, such as amino compounds free from carboxyl groups. The addition of the last-mentioned agents has the effect that inorganic impurities, such as those which are present in the hardness components of water and in technical grade metal salts, will not have a detrimental effect upon the brightening effect.

Amino compounds free from carboxyl groups of this type are, for example, N,N,N',N'-tetraethyl-1,3-diaminopropanol-2; N,N,N',N'-tetrahydroxyethyl-ethylene - diamine-2 - diethylamino-ethylchloride - 1; N,N - dimethyl - 4-bromoanilin-3-diethylamino-1-chloropropanol-2; as well as halogen salts of quaternary ammonium compounds which have been formed from the last-mentioned substituents by internal rearrangement, as well as sulfuric acid derivatives which are derived from the first-mentioned amino compounds, such as N,N,N',N'-tetra-n-butyl-1,3-diaminopropanol-2-monosulfuric acid ester and piperazine-N,N'-bis-(2-hydroxypropane-sulfonic acid).

The brightening agents according to the invention may also be advantageously used in an acid direct copper plating process, that is a process in which the metal objects are treated prior to electroplating in an acid pickling bath containing inhibitors with a high inhibiting effect, and subsequently directly electroplated in said copper baths containing the agents according to the invention, without intermediate rinsing.

The brightening agents according to the invention may be used in acid, cyanide and alkaline electroplating baths for the production of copper, zinc, cadmium, tin, brass, bronze, silver and gold electroplates. The brightening agents are added to the baths in quantities from 0.001 gm./liter to 5 gm./liter, preferably from 0.05 to 0.03 gm./liter, and the electroplating process is carried out at bath temperatures from room temperature to 60° C., in alkaline baths up to 90° C., and in current density ranges from 0.5 amp./dm.<sup>2</sup> to 16 amp./dm.<sup>2</sup>, in alkaline baths up to 40 amp./dm.<sup>2</sup>.

The following examples are set forth to enable persons skilled in the art to better understand and practice our invention and are not intended to be limitative.

#### Example I

A customary acid copper electroplating bath which contained 210 gm./liter CuSO<sub>4</sub>·5H<sub>2</sub>O, 60 gm./liter H<sub>2</sub>SO<sub>4</sub> and as brightening agent 2 gm./liter of a condensation product of dodecylalcohol and 10 mols ethylene oxide, which had been 25% transformed into the sulfuric acid ester, was modified with 0.3 gm./liter of the sodium salt of caprothiolactam-N-(propane-ω-sulfonic acid) having the structural formula



and 2 gm./liter 2-N-diethylamino-ethylchloride having the structural formula



Full bright, ductile copper electroplates, were obtained on metallic bases, such as iron, steel, brass or also copper, within a current density range of 0.5 to 7.5 amp./dm.<sup>2</sup> at 10 to 29° C.

#### Example II

The following products, which were used in the form of their alkaline metal salts, with the same effect as the

brightening agent for the acid copper bath illustrated in Example I:

|    | Brightening Agent                                                                                                   | gm./liter |
|----|---------------------------------------------------------------------------------------------------------------------|-----------|
| 5  | Thioacetamide-N-(propane-ω-sulfonic acid).....                                                                      | 0.3       |
|    | Thioacetamide-N-(methane sulfonic acid).....                                                                        | 0.05-0.2  |
|    | Thioformamide-N-(butane-ω-sulfonic acid).....                                                                       | 0.2       |
|    | Thioacetamide-N-butyl-N-(propane-ω-sulfonic acid).....                                                              | 0.3       |
| 10 | Thioacetamide-N-cyclohexyl-N-(propane-ω-sulfonic acid).....                                                         | 0.25      |
|    | Thioacetamide-N-benzyl-N-(propane-ω-sulfonic acid).....                                                             | 0.1-0.2   |
|    | Thiobenzamide-N-(propane-ω-sulfonic acid).....                                                                      | 0.2       |
|    | Thiopicolinic acid - N - methyl - N - (propane - ω - sulfonic acid)-amide-N'-(propane-ω-sulfonic acid)-betaine..... | 0.3       |
| 15 | Thiopicolinic acid - N - phenyl - N - (propane - ω - sulfonic acid)-amide-N'-(propane-ω-sulfonic acid)-betaine..... | 0.3       |
|    | Ethylene - 1,2 - bis - [thioacetamide - N,N' - bis (propane-ω-sulfonic acid)]-N,N'.....                             | 0.05      |
|    | N - (propane - ω - sulfonic acid) - thioacetimino - S - ethyl-ester.....                                            | 0.1       |
|    | N-(propane-ω-sulfonic acid)-thioacetimino-S-propylester.....                                                        | 0.1       |
|    | N-(butane-ω-sulfonic acid)-thiobenzimino-S-n-butylerster.....                                                       | 0.2-0.3   |
|    | N-(propane-ω-sulfonic acid)-thioacetimino-S-benzylester.....                                                        | 0.1       |
| 20 | N - (propane - ω - sulfonic acid) - thioacetimino - S - (p-chlorophenyl) ester.....                                 | 0.4       |
|    | N-(2-hydroxypropane-ω-sulfonic acid)-thiobutyrimino-S-cyclohexylester.....                                          | 0.8       |
|    | N - (propane - ω - sulfonic acid) - 2 - hydroxythiobenzimino-S-ethylester.....                                      | 0.6       |

#### Example III

Sheet iron or sheet steel was electroplated in an acid zinc electroplating bath which contained 200 gm./liter zinc sulfate, 0.5 to 2 gm./liter glacial acetic acid and, as brightening agent, 1.5 gm./liter thioacetamide-N-methane sulfonic acid within the current density range of 1 to 6 amp./dm.<sup>2</sup> and at room temperature. Bright zinc electroplates were obtained. Without the above brightening agent additive the zinc electroplates are dull under otherwise identical conditions.

#### Example IV

A zinc electroplating bath containing 56.5 gm./liter zinc cyanide, 71.5 gm./liter sodium hydroxide and 40.3 gm./liter sodium cyanide was modified with 1 to 2 gm./liter of the sodium salt of thioformamide-N-(toluene-2-sulfonic acid). Iron or steel objects electroplated in this bath between room temperature and above 40° C. at a current density from 1 to 24 amp./dm.<sup>2</sup> were provided with a bright zinc electroplate. Without the addition of the thioformamide derivative brownish discolored zinc electroplates were obtained.

#### Example V

A cadmium bath containing 135 gm./liter cadmium sulfate, 145 gm./liter sodium cyanide and 70 gm./liter caustic soda was modified with 2.5 gm./liter of the sodium salt of N-(propane-ω-sulfonic acid) - thioacetimino - S-benzylester. Iron or steel objects electroplated in this bath at room temperature and a current density from 1 to 5 amp./dm.<sup>2</sup> were provided with bright cadmium electroplates.

#### Example VI

Uniform brass electroplates on iron and steel objects were obtained when these materials were electroplated in a bath which contained 30 gm./liter copper cyanide, 60 9.4 gm./liter zinc cyanide, 56 gm./liter sodium cyanide, 30 gm./liter N-hydro soda and, as brightening agent, 0.5 gm./liter of the sodium salt of thiopropionamide - N-(naphthalene-8-sulfonic acid). The electroplating process was advantageously carried out at 50 to 60° C. at 65 current densities of 1 to 4.5 amp./dm.<sup>2</sup>. By further adding 1.2 gm./liter of the sodium salt of ethylene-1,2-bis[thioacetamide - N,N'-bis - (butane - ω - sulfonic acid)] the uniform brass electroplates became full-bright.

#### Example VII

A tin electroplating bath which contained 420 gm./liter potassium stannate and 22.5 gm./liter potassium hydroxide was modified with 3.5 gm./liter of potassium salt of caprothiolactam-N-(propane-ω-sulfonic acid). At current densities of 2 to 40 amp./dm.<sup>2</sup> and at temperatures

from 50 to 90° C., iron or steel objects were provided with full bright tin electroplates.

*Example VIII*

Thioacetamide - N - (propane -  $\omega$  - sulfonic acid) sodium salt having the following structural formula:



may be prepared by the following method. 16.1 gm./liter (0.1 mol)  $\omega$ -aminopropane-sodium sulfonate and 7.5 gm. (0.1 mol) thioacetamide were dissolved in 50 cc. water and the solution was heated for some time to 80° C., whereby ammonia escaped. After the evolution of ammonia had ceased the solution was evaporated in a vacuum. 20.7 gm. of a greenish-yellow product remained as a residue, which was purified by dissolving it in a small amount of water and reprecipitating it by adding an ether-acetone mixture. The use of this compound as a brightening agent is illustrated in Example II.

*Example IX*

The sodium salt of N-(propane- $\omega$ -sulfonic acid)-thioacetimino-S-benzylester having the following structural formula:



may be prepared by the following method. 20.1 gm. of the hydrochloride of thioacetamino-S-benzylesters were dissolved in 100 cc. water and the solution was added dropwise at 60° C. to a solution of 24.4 gm. propane sulfone in 50 cc. ethanol. The turbid reaction solution was maintained for 2 hours at a temperature of 60 to 70° C., accompanied by stirring. After cooling, the solution was neutralized with aqueous sodium hydroxide. Subsequently, in order to remove components having a bad odor, the solution was extracted with ether. The aqueous solution of the sodium salt of N-(propane- $\omega$ -sulfonic acid)-thioacetimino-S-benzylester is employed as illustrated in Example II.

While we have set forth specific embodiments and preferred modes of practice of our invention, it will be understood that we do not intend to be limited thereby, and that various changes and modifications may be made within the spirit of the invention and the scope of the appended claims.

We claim:

1. A method for producing bright metal electrodeposits on a base metal, which comprises adding as a brightening compound to the electroplating bath solution containing a compound of the metal to be electrodeposited, a sulfonic acid compound having a structural formula, selected from the group consisting of:



and



and their alkali metal salts, wherein R and R' are selected from the group consisting of hydrogen, hydrocarbon radicals, and taken together a polymethylene chain of a heterocyclic ring, and R'' is a hydrocarbon radical, said brightening agent being added in sufficient amount to obtain said bright electrodeposits.

2. The process of claim 1 wherein the electroplating bath is selected from the group consisting of acid, cyanide and alkaline baths.

3. The process of claim 1 wherein amino compounds free from carboxyl groups are added to the electroplating bath.

4. A method for producing bright metal electrodeposits on a base metal, which comprises adding as a brightening compound to the electroplating bath solution containing a compound of the metal to be electrodeposited, a sulfonic acid compound having a structural formula, selected from the group consisting of:



and



25 and their alkali metal salts, wherein R and R' are selected from the group consisting of hydrogen, hydrocarbon radicals, and taken together a polymethylene chain of a heterocyclic ring, and R'' is a hydrocarbon radical, and in addition compounds having a structural formula selected from the group consisting of



and



wherein R, R' and R'' represent groups as above defined, said brightening agent being added in sufficient amount to obtain said bright electrodeposits.

5. A method for producing bright copper electrodeposits on a base metal, which comprises adding as a brightening compound to an acid copper electroplating bath solution a sulfonic acid compound having a structural formula, selected from the group consisting of:



and



60 and their alkali metal salts, wherein R and R' are selected from the group consisting of hydrogen, hydrocarbon radicals, and taken together a polymethylene chain of a heterocyclic ring, and R'' is a hydrocarbon radical, said brightening agent being added in sufficient amount to obtain said bright electrodeposits.

6. The method of claim 1 wherein the amount of brightening compound added is from about 0.001 to about 5 g./l.

7. An electroplating bath for producing bright metal electrodeposits on base metals which comprises an aqueous solution of a compound of the metal to be deposited and a brightening compound which is a sulfonic

7  
acid compound having a structural formula, selected from  
the group consisting of:



and



and their alkali metal salts, wherein R and R' are selected from the group consisting of hydrogen, hydrocarbon radicals, and taken together a polymethylene chain of a heterocyclic ring, and R'' is a hydrocarbon radical, said brightening agent being added in sufficient amount to obtain said bright electrodeposits.

8. An electroplating bath as defined in claim 7 selected from the group consisting of acid, cyanide and alkaline baths.

9. The bath of claim 7 wherein said electroplating bath contains in addition amino compounds free from carboxyl groups.

10. An electroplating bath for producing bright metal electrodeposits on base metals which comprises an aqueous solution of a compound of the metal to be deposited, a brightening compound which is a sulfonic acid compound having a structural formula, selected from the group consisting of:



and



and their alkali metal salts, wherein R and R' are selected from the group consisting of hydrogen, hydrocarbon radicals, and taken together a polymethylene chain of a heterocyclic ring, and R'' is a hydrocarbon radical, and in addition compounds having a structural formula selected from the group consisting of



and



5  
wherein R, R' and R'' represent groups as above defined, said brightening agent being added in sufficient amount to obtain said bright electrodeposits.

11. An acid copper electroplating bath for directly producing bright copper electrodeposits on base metals which comprises an aqueous acid solution of a copper salt and a brightening compound which is a sulfonic acid compound having a structural formula, selected from the group consisting of:



15  
and



25  
and their alkali metal salts, wherein R and R' are selected from the group consisting of hydrogen, hydrocarbon radicals, and taken together a polymethylene chain of a heterocyclic ring, and R'' is a hydrocarbon radical, said brightening agent being added in sufficient amount to obtain said bright electrodeposits.

30  
35  
12. The bath of claim 7 wherein the amount of brightening compound added is from about 0.001 to about 5 gm./liter.

#### References Cited in the file of this patent

#### UNITED STATES PATENTS

|                |                        |                                                                                         |                                                                                                                                                                   |                                                                                                                    |                                                      |
|----------------|------------------------|-----------------------------------------------------------------------------------------|-------------------------------------------------------------------------------------------------------------------------------------------------------------------|--------------------------------------------------------------------------------------------------------------------|------------------------------------------------------|
| 2,489,538      | Phillips et al. -----  | Nov. 29, 1949                                                                           |                                                                                                                                                                   |                                                                                                                    |                                                      |
| 2,663,684      | Pierce -----           | Dec. 22, 1953                                                                           |                                                                                                                                                                   |                                                                                                                    |                                                      |
| 2,742,413      | Cransberg et al. ----- | Apr. 17, 1956                                                                           |                                                                                                                                                                   |                                                                                                                    |                                                      |
| 2,772,309      | Doerner -----          | Nov. 27, 1956                                                                           |                                                                                                                                                                   |                                                                                                                    |                                                      |
| 2,806,879      | Kaiser et al. -----    | Sept. 17, 1957                                                                          |                                                                                                                                                                   |                                                                                                                    |                                                      |
| 2,830,014      | Gundel et al. -----    | Apr. 8, 1958                                                                            |                                                                                                                                                                   |                                                                                                                    |                                                      |
| 40<br>45<br>50 | 40<br>45<br>50         | 2,837,472<br>2,849,351<br>2,849,352<br>2,903,403<br>2,905,602<br>2,937,978<br>2,950,235 | Gundel et al. -----<br>Gundel et al. -----<br>Kirstahler et al. -----<br>Strauss -----<br>Kirstahler et al. -----<br>Strauss et al. -----<br>Strauss et al. ----- | June 3, 1958<br>Aug. 26, 1958<br>Aug. 26, 1958<br>Sept. 8, 1959<br>Sept. 22, 1959<br>May 24, 1960<br>Aug. 23, 1960 | 1958<br>1958<br>1958<br>1959<br>1959<br>1960<br>1960 |

UNITED STATES PATENT OFFICE  
CERTIFICATE OF CORRECTION

Patent No. 3,075,899

January 29, 1963

Wennemar Strauss et al.

It is hereby certified that error appears in the above numbered patent requiring correction and that the said Letters Patent should read as corrected below.

Column 3, line 38, for "0.03" read -- 0.3 --.

Signed and sealed this 3rd day of September 1963.

(SEAL)

Attest:

ERNEST W. SWIDER  
Attesting Officer

DAVID L. LADD  
Commissioner of Patents